

## UNITED STATES PATENT OFFICE

LUDWIG KERN, OF WEBSTER GROVES, MISSOURI

## FUEL AND THE MANUFACTURE THEREOF

No Drawing.

Application filed June 18, 1930. Serial No. 462,130.

This invention relates to fuels, and with regard to certain more specific features, to liquid fuels of low specific gravity.

Among the several objects of the invention 5 may be noted the provision of fuel such as a fuel oil, the calorific value of which has been enhanced by the addition of porous, light carbonaceous particles in substantially permanent suspension; a fuel of the class described which is economically prepared; the provision of a process for manufacturing 10 from carbonaceous materials a porous, voluminous powder which will remain in suspension in liquids such as oil for lengthy periods of time; a process of the class described which additionally provides for the removal 15 of sulphur and the like from the carbonaceous material in the course of its preparation into said voluminous powder; and a process 20 of the class described which is easily and economically carried through with a minimum of costly treating materials. Other objects will be in part obvious and in part pointed out hereinafter.

25 The invention accordingly comprises the elements and combinations of elements, steps and sequence of steps and features of synthesis which will be exemplified in the description hereinafter and the scope of the application of which will be indicated in the following claims.

The present invention is concerned with the production of a liquid fuel of higher calorific value than heretofore had. This additional calorific value is secured by suspending within the fuel oil a carbonaceous solid material, light in specific gravity and in a state of subdivision such that it will remain in substantially permanent suspension within the liquid oil. Ordinary pulverized bituminous or carbonaceous materials are too heavy, and settle out of suspension in a short time, thereby rendering such materials ineffective for the present purposes. I have found, however, a method for forming a highly porous, low specific gravity, voluminous carbon powder from distillable carbonaceous materials such as bituminous coal, sub-bituminous coal, semi-bituminous coal, anthracite, lignite, culm, and other materials

of a similar nature. The process referred to is set forth hereinafter:

The carbonaceous material is first ground to a fineness of the order of 200 mesh or finer, at which fineness the ash-forming constituents are mechanically detached from the carbon constituents. The comminuted carbonaceous material is then masticated or homogenized in a pug mill or the like with water in order to form said material into a loose but plastic, cohesive mass. This is accomplished by the mixing of the pulverized ash-forming constituents and water to form a binder material for the carbon constituents. Pressing of the plastic mass is avoided so far as practicable.

The wet, plastic mass is next conveyed into a retort, and rapidly brought to a temperature of the order of 550° C. or lower, at which temperature the water and volatiles in the carbonaceous material are vaporized with almost explosive violence, and the material is inflated to form a highly porous, voluminous mass. The products of distillation are recovered and condensed by methods customary to the art. It is desirable to leave at least a part of the volatiles in the carbonaceous material, to aid in effecting a suspension in oil as hereinafter described.

After the distillation is complete, the de-volatilized mass is allowed to cool, preferably with exclusion of air to prevent combustion. The cooled mass is not spontaneously combustible, however, and may be handled in air without danger.

The cooled product is then subjected to a grinding to reduce it to a fineness of the order of 200 mesh. The finest particles are preferably separated by air flotation. The porous, highly voluminous product is then packaged for use in a customary manner.

In the case of carbonaceous materials which have a high sulphur content, it is desirable that dilute aqueous hydrochloric acid solutions (from 2 to 5° Bé.) or chloride solutions, preferably magnesium chloride solutions (from 2 to 5° Bé.) be used in place of water in the plasticizing operation. In this case the chloride, or the hydrogen evolved by reactions of the chlorides with the water pres-

ent under the catalytic influence of the ash-forming constituents, or the hydrogen obtained by decomposition of the hydrochloric acid, unite with the sulphur and are vaporized with the other volatiles as hydrogen sulphide or sulphur chlorides or the like. Sulphur is thus removed and the voluminous powder is substantially sulphur-free.

The voluminous carbon powder obtained has a specific gravity ranging from 0.30 to 0.50. This powder is now mixed into a fuel oil. Fuel oils generally range in specific gravity from 0.70 to 0.90. It will be seen that the carbon powder will not settle from its suspension in the oil, but will rather float in the oil. The lightness of particle and fineness of particle size, together with the residual volatiles in the powder, coact to effect a substantially permanent suspension of the carbon powder in the oil. The carbon powder, having a high calorific value, enhances the calorific value of the combined fuel over that of the fuel oil alone. The smallness of carbon particle size further permits the oil to be sprayed as is customary in fuel oil burners, and to burn rapidly and completely.

In view of the foregoing, it will be seen that the several objects of the invention are achieved and other advantageous results attained.

As many changes could be made in carrying out the above objects without departing from the scope of the invention, it is intended that all matter contained in the above description shall be interpreted as illustrative and not in a limiting sense.

I claim:

1. The liquid fuel comprising a fuel oil of specific gravity from 0.70 to 0.90, said oil having in suspension therein a carbon powder of a fineness greater than the order of 200 mesh and a gravity of the order of from 0.30 to 0.50.

2. The process of preparing a liquid fuel which comprises forming a porous, light carbon powder in the following manner: comminuting carbonaceous distillable material, plasticizing said comminuted material with water, and rapidly heating said plastic material to a carbonization temperature, whereby said material is inflated, cooling said inflated material and pulverizing the same; and mixing said carbon powder with fuel oil whereby a substantially permanent suspension is obtained.

3. The method of manufacturing a porous, voluminous carbon powder which comprises pulverizing coal to a fineness of the order of 200 mesh, thereby mechanically detaching the ash-forming constituents from the carbonaceous constituents of said coal, plasticizing said ash-forming constituents with water whereby said coal mass is rendered plastic, heating said plastic mass rapidly to a

temperature of the order of 550° C., whereby volatile constituents of said coal and said water are rapidly evolved and said plastic material is inflated, cooling said inflated material and grinding the same.

4. The method of manufacturing a porous, voluminous carbon powder which comprises pulverizing coal to a fineness of the order of 200 mesh, thereby mechanically detaching the ash-forming constituents from the carbonaceous constituents of said coal, plasticizing said ash-forming constituents with acids whereby said coal mass is rendered plastic, heating said plastic mass rapidly to a temperature of the order of 550° C., whereby volatile constituents of said coal and said water are rapidly evolved and said plastic material is inflated and sulphur constituents are volatilized, cooling the inflated material and grinding the same.

5. The method of manufacturing a porous, voluminous carbon powder which comprises pulverizing coal to a fineness of the order of 200 mesh, thereby mechanically detaching the ash-forming constituents from the carbonaceous constituents of said coal, plasticizing said ash-forming constituents with chloride solutions whereby said coal mass is rendered plastic, heating said plastic mass rapidly to a temperature of the order of 550° C., whereby volatile constituents of said coal and said water are rapidly evolved and said plastic material is inflated and sulphur constituents are volatilized, cooling the inflated material and grinding the same.

6. The process of preparing a liquid fuel which comprises forming a porous, light carbon powder in the following manner: comminuting carbonaceous distillable material, plasticizing said comminuted material, and rapidly heating said plastic material to a carbonization temperature, whereby said material is inflated, cooling said inflated material and pulverizing the same; and mixing said carbon powder with fuel oil whereby a substantially permanent suspension is obtained.

In testimony whereof, I have signed my name to this specification this 13th day of June, 1930.

LUDWIG KERN.

70

75

80

85

90

95

100

105

110

115

120

125

130